

May 17, 1932.

I. SILBERSTEIN

1,859,112

METHOD OF MANUFACTURING ELECTRICAL RESISTANCES

Filed Dec. 11, 1929

Fig. 1



Fig. 2



Inventor:  
Isidor Silberstein  
by Parker + Carter.  
Attorneys.

## UNITED STATES PATENT OFFICE

ISIDOR SILBERSTEIN, OF BERLIN, GERMANY

## METHOD OF MANUFACTURING ELECTRICAL RESISTANCES

Application filed December 11, 1929, Serial No. 413,167, and in Germany December 18, 1928.

My invention relates to improvements in the method of manufacturing electrical resistances, and more particularly in the method in which a resistance material is applied to a suitable carrier and portions are cut therefrom to leave a strip of the desired resistance on the carrier. The object of the improvements is to provide a method by means of which exact resistances are produced, and 10 with this object in view my invention consists in first coating the resistance material initially applied to the carrier with a protective layer such as lacquer adapted to prevent injury to the resistance material by chips 15 or powder cut from the body of resistance material and the carrier. Other objects of the improvements will appear from the following description.

For the purpose of explaining the invention a resistance and an apparatus suitable for manufacturing the same have been shown in the accompanying drawings, in which

Fig. 1 is an elevation partly in section showing a resistance, and

Fig. 2 is a diagrammatical elevation partly in section showing the apparatus for manufacturing the resistance.

The resistance illustrated in Fig. 1 comprises a carrier 1 of insulating material such as ceramic material, a resistance strip 2 applied to the said carrier, a coating 3 of lacquer or other non-conductive material, and terminals 10 in the form of caps fixed to the ends of the carrier and electrically connected with the resistance material. The strip 2 of resistance material is bounded at both sides by grooves 4 cut into the carrier. In the example shown in Fig. 1 the resistance strip is in the form of a helix laid around the cylindrical core 1.

In the manufacture of the resistance I proceed as follows: The carrier 1 is first coated with the resistance material 2, which may be for example a material containing carbon, 45 as is known in the art. The coated core is

now exactly measured, and from the dimensions thus obtained the breadth and the pitch of the helical line 4 to be ground into the protective coating, the resistance material and the core are exactly calculated so as to obtain the desired resistance. The blank thus prepared is placed on a lathe, and the terminals 10 of the carrier 1 are connected with a source of electric energy and an apparatus for measuring current intensities. Preferably I use an apparatus such as an ammeter the scale marks of which directly indicate resistances. Now the groove 4 is cut into the blank while observing the current intensity or resistance indicated by the ammeter, the grinding operation being interrupted when the desired resistance is obtained. Thus by measuring the resistance in the course of the grinding operation the desired resistance is obtained.

In Fig. 2 I have shown an apparatus in the form of a lathe suitable for cutting the groove 4. In the said figure the blank to be ground has received the reference character 12, which blank is placed on the centers 5 of the lathe for being rotated thereby. The said centers are engaged by brushes 6 disposed in a circuit including a source of electric energy 7 and an ammeter 8 or similar measuring instrument. The centers 5 are insulated from the spindles of the lathe by means of insulating blocks 11. For grinding the helical groove on the blank a rotary grinding disk 9 is provided, which is mounted on a suitable slide-rest 13 by means of which it is adapted to be shifted in the direction of the arrow  $\alpha$  while rotating the blank. Thus a helical groove 4 of the desired pitch is cut through the protective coating 3, the resistance material 2 and into the core 1, while the ammeter 8 is observed, the operation being interrupted when the ammeter shows the desired resistance.

By first coating the resistance material with a protective layer I am enabled to pro-

duce an exact cut of the resistance strip, the said resistance strip being held while grinding between the protective layer and the carrier, and any injury to the resistance material by chips cut from the ceramic material is made impossible.

After cutting the resistance in the manner described I coat the blank with a suitable insulating lacquer by means of which any excess of air or moisture to the resistance material is prevented and the previous insulation of the resistance material is reestablished.

In my improved method the waste caused by failure in the manufacture is reduced to a minimum, so that the manufacture is economical.

In the preferred method the carrier 1 of ceramic or other insulating material is first ground exactly to the desired diameter before applying the insulating and protective coatings thereto. By thus producing an exactly cylindrical blank the grinding operation is made more satisfactory and more exact.

While in describing the invention reference has been made to a resistance strip in the form of a helix I wish it to be understood that my invention is not limited to the form of the strip shown in the figures, and that various other forms may be made on the carrier. For example I may grind the blank so that a system of straight and parallel resistance strips is produced. Further, the strip may be ground with varying pitch, and a plurality of helical strips may be provided one beside the other.

I claim:

1. The herein described method of manufacturing electrical resistances, which consists in applying a coating of resistance material to a carrier of insulating material, applying thereto a protective coating, and thereafter removing portions of the said coatings to produce the resistance in the desired form.

2. The herein described method of manufacturing electrical resistances, which consists in applying a coating of resistance material to a carrier of insulating material, applying thereto a protective coating, and thereafter cutting from the said layers portions so as to leave resistances of the desired form.

3. The herein described method of manufacturing electrical resistances, which consists in applying a coating of resistance material to a carrier of insulating material, applying thereto a protective coating, and thereafter grinding from the said layers and the surface of the carrier portions so as to leave resistances of the desired form.

4. The herein described method of manufacturing electrical resistances, which consists in applying a coating of resistance ma-

terial to a carrier of insulating material, applying thereto a protective coating, and thereafter grinding through the protective layer, the resistance material and into the carrier a helical groove of a shape suitable for leaving a coating of the desired resistance on the carrier.

Signed at Berlin, this 25th day of November, 1929.

ISIDOR SILBERSTEIN. 75

80

85

90

95

100

105

110

115

120

125

129